

Nov. 2, 1943.

A. M. LANDESMAN ET AL  
METHOD OR PROCESS FOR THE REPAIR OF BROKEN OR  
DAMAGED GLASSWARE AND THE LIKE  
Filed Jan. 10, 1942

2,333,186



FIG. 1.



FIG. 2.



FIG. 3.



FIG. 4.



FIG. 5.

INVENTORS  
ALFRED M. LANDESMAN  
EUGENE LANDESMAN

By *Alfred Landesman*  
ATTORNEY

## UNITED STATES PATENT OFFICE

2,333,186

METHOD OR PROCESS FOR THE REPAIR OF  
BROKEN OR DAMAGED GLASSWARE AND  
THE LIKEAlfred M. Landesman and Eugene Landesman,  
St. Louis, Mo.

Application January 10, 1942, Serial No. 426,302

6 Claims. (Cl. 49—82)

This invention has to do with, and has for its objects and resides in the provision of, a certain new, useful, and unique method or process which may with economy and facility be practiced for the repair of broken glassware and the like.

Broadly stated, our invention contemplates the fitting together of the several pieces or fragments of a broken article of glassware to their initial or, as may be said, setting the major and minor portions, parts, or fragments of the broken glassware article into their original relationship; substantially enveloping the article, with the major and minor broken pieces, parts, or fragments so disposed, in a refractory paste and permitting the paste to set and harden for maintaining such parts or fragments in fitted, initial or original relation and for preserving their original form and contour during subjection thereof to heat, such parts or fragments along and adjacent the juncture line or lines or joints therebetween being preferably clear of the refractory material, however, on their outer face for purposes presently appearing; disposing the article so encased in the set or hardened refractory material within a furnace of unique structure and gradually or slowly raising the temperature within the furnace to a safety working state, which may vary within a range presently set forth, depending upon the glass-structure being worked or repaired; applying greater or more intense heat by means of a torch, blow-pipe, or other suitable instrument or tool directly on the article portions or fragments along and adjacent the juncture line or lines or joints therebetween and thereby substantially fusing or integrating the same at and along such lines; permitting the furnace and the work to gradually or slowly cool to substantially room temperature, when the article, being then removed from the furnace and subjected to water for effecting the removal of the hardened refractory coating, is presented to view restored to substantially or approximately initial, original, or unbroken condition.

In practicing our glassware repair process or method, we make use of certain equipment, which, for clarifying the steps of our method, we portray in the accompanying drawing, in which—

Figure 1 is a perspective view illustrating a broken article of glassware with its major and minor portions or parts in juxtaposed relation and the repair and restoration of which to substantially initial or original condition is to be

effected in accordance with the method or process of our invention or discovery;

Figure 2 illustrates the article of Figure 1 with its major and minor fragments in fitted or assembled approximately initial relation and substantially completely enveloped in a refractory material except upon its outer face at and adjacent the juncture lines or joints between the major and minor parts or fragments for hardening of the refractory material and for disposition within the heating oven or furnace;

Figure 3 is a reduced illustration of a heating oven or furnace of unique form and structure employed in the practicing of our invention;

Figure 4 illustrates the disposition within the furnace through openings provided therein for the purpose of a torch, blow-pipe, or other suitable instrument or tool for raising the temperature of the article at the juncture line or lines between the fragments thereof to such a relatively high degree as to effect substantial fusing together along such lines only of the article portions or parts; and

Figure 5 is a perspective view of the repaired article.

Referring now more in detail and by reference characters to the accompanying drawing, A designates a glass vase, goblet, or the like of any suitable form and of any usual, ordinary, or common glass structure or composition, which, accidentally or otherwise, has been broken into a so-called major portion *a* and minor fragments *a'*, for effecting the permanent restoration of which to substantially original or initial condition our invention is particularly adapted.

It is a relatively simple matter to substantially cover the complete article with a layer of suitable thickness, usually one-quarter inch, of a refractory paste or material of suitable consistency and to hold the parts in substantially their original relation until the refractory material sets sufficiently to retain the parts in such original relation, the dry or set material then functioning substantially as a mold, should the glass become soft at any stage of the process. The refractory paste is, of course, carefully omitted from between the several parts or fragments, and while the refractory paste may substantially completely cover the several parts or fragments and the cracks therebetween, we prefer to leave a small quarter-inch area on both sides the cracks on one face free from the refractory paste. This makes it possible to heat the glass to a higher degree of temperature with-

out the refractory material dulling the glass when the intense heat is applied.

The refractory material B that we preferably employ in the practicing of our invention is initially in the form of an impalpable powder comprising as its ingredients approximately twenty-five parts of plaster of Paris, seventy-four parts of silica, and eight-tenths part of sodium chloride, all thoroughly mixed and commingled, sufficient water being added at time of application to make a paste of the desired consistency.

While we prefer to employ a refractory material B of the composition named, it will be understood that any other material suitable for the purpose may be equally well used, it being only essential that the material be of such a nature as not to chemically react with the glass at any time and as to have the properties and characteristics of being capable of (1) withstanding, when set and hard, relatively high temperatures ranging up to approximately 2000° F., and have a coefficient of expansion comparable to that of the glass-structure of the article A being repaired, so as, when heated, to eliminate the exertion upon the article of any extraordinary stresses that might disrupt, break, or otherwise damage the encased article A, and (2) ready removal by cracking or otherwise following completion of the repair operation mentioned and presently described more in detail.

Such refractory material is also initially, as we have stated, in the form of a powder and may be mixed with a suitable vehicle, such, for instance, as water, for convenient application upon the article A in the form of a paste of the desired consistency, as we have mentioned, and which will subsequently dry or set without material shrinkage and without exerting any impairing or damaging stresses upon the article A being repaired.

The article A, so encased and supported by means of the refractory material, is allowed to set and stand over a relatively long period of time, approximately twenty-four hours, for enabling air-drying of the material B, and when the material B has become thoroughly dry and set, the article A is placed in a heating furnace or oven D of any suitable standard or common form or type, with the exception that the body d of the oven or furnace D is provided with a plurality of sets of openings or apertures 6, 6', the openings of each pair being spaced more or less closely together for purposes presently appearing.

We might here state that the oven or furnace D is heated by any suitable means capable preferably of precise and accurate control, and for such purpose we have found that electric heating elements C lend themselves efficiently to the requirements of precise control advantageous in the practicing of our process. In this same connection, it may be remarked that the oven or furnace D is preferably of any suitable relatively small-size refractory brick type, except, as we have stated, that the furnace D, in the walls of its body d, should be breached in a number of convenient places for providing suitable openings or apertures 6, 6', of such dimensions as to afford vision into the furnace and insertion thereinto of a torch, blow-pipe, or other suitable heating instrument or tool E for working the glass-structure of the article A being treated or repaired. We might add that it is most convenient that such apertures or openings 6, 6', be in pair relation, so that the operator may observe the work through one aperture while manipulating

the torch E through the other, the apertures or openings 6, 6', being sufficiently large to permit a certain amount of freedom for torch or blow-pipe manipulation.

5 The number and position of such openings or apertures 6, 6', depend upon the desires and skill of the workmen and should be located so that objects A of various types and sizes disposed within the oven or furnace D may be readily accessible for torch or blow-pipe working, it being, of course, obvious that the article A, when disposed in the oven or furnace D, should be positioned in such a manner that the preferably exposed break lines or cracks or joints between the portions a and a' thereof will face, and be accessible by means of the torch, blow-pipe, or the like E through, one or more of such apertures or openings 6, 6'.

20 The temperature of the oven or furnace D is now slowly or gradually raised to so-called safety range anywhere from 800° F. to 1500° F., depending upon the nature and glass-structure of the article A. The initial heating should, of course, be performed so as to prevent the breaking or 25 cracking of the glass object under repair, and it may be here remarked that some glassware may be brought up to such safety range in less time than others and that a workman familiar with glassware will be readily able to determine by 30 inspection the type of glassware and the approximate range at which the glass may be safely heated. Experience with a wide variety of glassware has indicated that a fairly safe heating range will comprise an initial elevation of about 35 50° per hour for the first four hours and a subsequent elevation of about 100° per hour for the next six or eight hours, the oven temperature being brought up, as we have stated, to a range of from 800° F. to 1500° F., depending upon the 40 glass-structure of the article A being repaired. We might remark that the optimum temperature which should be reached may be termed the safety range, and, again, such range will vary for different glassware. Experience, however, 45 has shown that, for all practical purposes, this heating will fall within the range of from 800° F. to 1500° F., depending upon the nature and glass-structure, that is to say, the formula, or composition of the particular article A of glassware 50 being treated. We might remark further that it has been found by extensive experiment that practically all types of standard or common glassware may be heated within the range mentioned without cracking or breaking, although it will, 55 of course, be understood that a glass-worker of experience and skill may readily determine the type or structure of glass which is being repaired and immediately associate with such glass some particular stage within the stated range which is most suited for the purposes in hand.

60 In any event, entirely satisfactory results may be attained within the range outlined, and once the article A has been brought up to the so-called safety range, a lighted blow-pipe, torch, or other suitable tool E is inserted through one of the apertures or openings 6, 6', in the wall d of the oven D and the flame thereof applied by the operator back and forth along the various cracks or joints between the exposed article-portions 65 a, a', the temperature of the exposed parts of the article A being thereby raised to the fusing or coalescing point, which may range anywhere 70 from 1500° F. to 2500° F., depending upon the nature and composition of the glass-structure of the particular article A.

Necessarily this step in our process must be carefully performed, so as to prevent distortion or deformation of the glass at and around the joints between the parts or portions *a*, *a'*, the article being preferably so disposed as to eliminate any misplacing movement of the viscous glass, and the hard refractory coat provided by the material *B* for the covered portions of the article *A* functioning as a mold to efficiently maintain the form and contour thereof.

Where the breaks or cracks being repaired are small and the pieces or fragments *a*, *a'*, fit neatly together, the torch *E* should preferably have a tip *e* capable of emitting a very fine pointed flame. Where, on the other hand, the cracks or breaks are rough and ragged and marginally do not fit neatly together, a broader flame should be employed for effecting juncture therebetween. In ordinary cases, however, a standard hydrogen blowpipe or torch will yield a flame sufficiently hot and of sufficient size for accomplishing efficiently the desired purpose.

The article *A*, while being so treated or worked, is disposed to the vision of the workman through the adjacent aperture *6* or *6'*, as the case may be, and when the juncture lines between the fragments *a*, *a'*, of the article *A* have, through fusion or coalescence, substantially visually disappeared, the torch *E* is removed and the oven *D* then permitted to gradually cool to room temperature, when the refractory supported and repaired article *A'* is removed from the furnace *D*, immersed in water, which quickly effects a breaking down and removal of the set refractory material *B*, and again put to a useful purpose.

We may add that, where the object or article *A* is damaged in such a manner that a plurality of chips or fragments *a'* have been broken out, the damage may be referred to as a compound break-out. Again, the several chips or portions *a'* may fit neatly and accurately back into place, or there may be small parts missing, so that, when the available parts have been fitted back into place, there is still a small hole, such as that indicated at *a''* in Figure 2. In either case, the parts are fitted back into place as neatly and as precisely as possible and the article *A* completely invested, as we have described, care being taken to leave spaces within the investment material *B* in the region where the glass is missing, so that the glass will fuse into the empty spaces, as at *a''*, as well as coalesce across the close-fitting edges of the breaks. Where the lost parts are small, the repaired object *A'* will be substantially as good as new and the area in which the repair was made will not be disfiguring. Should the glass around the area that was fused become dull or even "bumpy" through or by application of excess heat, such defects may be readily removed by the usual means for grinding or polishing glass.

It should be understood that changes and variations in the steps of our process may be made and substituted for those herein set forth and described without departing from the nature and principle of our invention.

Having thus described our invention, what we claim and desire to secure by Letters Patent is,

1. That process of glassware repair which comprises fitting the major and minor parts of a broken glass article into original abutting relation, then by means of a refractory material disposed substantially completely over the major and minor parts of such article, except upon one side and at the line of abutment of said parts, approximately covering and encasing the article and

its major and minor parts within and by such refractory material, disposing the refractory-covered article within an oven, raising the temperature of the oven for preliminarily heating the housed article within a safety range, and then by means of a heating tool applying upon said parts or fragments more intense heat for fusing the same together.

2. That process of glassware repair which comprises fitting the major and minor parts of a broken glass article into original abutting relation, then disposing a refractory material in plastic form substantially completely over the major and minor parts of such article, except upon one side and at the line of abutment of said parts, permitting said plastic material to set and harden and thereby approximately covering and encasing the article and its major and minor parts in and by such plastic material, disposing the refractory-covered article within an oven, raising the temperature of the oven for preliminarily heating the housed article within a safety range, and then by means of a heating tool applied directly upon said exposed parts or fragments subjecting said parts or fragments to more intense heat for fusing the same together.

3. That process of glassware repair which comprises fitting the major and minor parts of a broken glass article into original abutting relation, then disposing a refractory material in plastic form substantially completely over the major and minor parts of such article, except upon one side and at the line of abutment of said parts, permitting the plastic material to set and harden and thereby approximately covering and encasing the article and its major and minor parts in and by such plastic material, disposing the refractory-covered article within an oven, raising the temperature of the oven for preliminarily heating the housed article within a safety range from 800° F. to 1500° F., and then by means of a heating tool applied directly upon said exposed parts or fragments subjecting said parts or fragments to a more intense heat ranging from 1500° F. to 2500° F. for fusing the same together.

4. That process of glassware repair which comprises fitting the major and minor parts of a broken glass article into original abutting relation, then disposing a refractory material in plastic form substantially completely over the major and minor parts of such article, except upon one side and at the line of abutment of said parts, permitting said plastic material to set and harden and thereby approximately covering and encasing the article and its major and minor parts in and by such plastic material, disposing the refractory-covered article within an oven, raising the temperature of the oven for preliminarily heating the housed article within a safety range, then by means of a heating tool applied directly upon said exposed parts or fragments subjecting said parts or fragments to more intense heat for fusing the same together, then permitting the article to gradually cool to room temperature, and then removing the refractory coating from the article.

5. That process of glassware repair which comprises fitting the major and minor parts of a broken glass article into original abutting relation, then by means of a refractory material disposed substantially completely over the major and minor parts of such article, except upon one side and at the line of abutment of said parts, approximately covering and encasing the article and its major and minor parts within and by such refractory material, disposing the encased article

within an oven and preliminarily heating the encased article within a safety range from 800° F. to 1500° F., then subjecting the encased article to a more intense heat ranging from 1500° F. to 2500° F. for fusing the broken parts thereof together, and then removing the article from the oven and displacing the refractory material.

6. That process of glassware repair which comprises fitting the major and minor parts of a broken glass article into original abutting relation, then by means of a refractory material disposed substantially completely over the major and minor parts of such article, except upon one side and at the line of abutment of said parts, ap-

proximately covering and encasing the article and its major and minor parts within and by such refractory material, disposing the encased article within an oven and preliminarily heating the encased article within a safety range from 800° F. to 1500° F., then subjecting the set parts of the encased article at the junctions therebetween to a more intense heat ranging from 1500° F. to 2500° F. for fusing the same together, and then removing the article from the oven and displacing the refractory material.

10

ALFRED M. LANDESMAN.  
EUGENE LANDESMAN.